

I. H. ELLSWORTH.  
PROCESS OF STRETCHING LEATHER.  
APPLICATION FILED FEB. 2, 1917.

1,235,299.

Patented July 31, 1917.



Fig. 1.

Fig. 2.



INVENTOR

Irving H. Ellsworth,  
By C. W. Owen & Crampton,  
His attorney.

# UNITED STATES PATENT OFFICE.

IRVING H. ELLSWORTH, OF ORRVILLE, OHIO.

## PROCESS OF STRETCHING LEATHER.

1,235,299.

Specification of Letters Patent. Patented July 31, 1917.

Application filed February 2, 1917. Serial No. 146,192.

To all whom it may concern:

Be it known that I, IRVING H. ELLSWORTH, a citizen of the United States, and a resident of Orrville, in the county of Wayne and

5 State of Ohio, have invented a certain new and useful Process of Stretching Leather; and I do hereby declare the following to be a full, clear, and exact description of the invention, such as will enable others skilled 10 in the art to which it appertains to make and use the same, reference being had to the accompanying drawings, and to the characters of reference marked thereon, which form a part of this specification.

15 This invention relates to the treatment of leather, and particularly to an improved process for stretching the same.

Leather is composed of more or less closely interwoven fibers and the pores or minute 20 spaces between the fibers are filled with the stuffing material which may comprise tallow, stearin, paraffin, wax, oils or the like, as well understood in the art. Stretching the leather lengthwise of the grain causes the 25 fibers thereof to fit more closely together and tends to force out the stuffing material if mellowed sufficiently for such purpose. The stuffing materials being solid, however, when in a cold state, remain to a greater or less 30 extent between the fibers during a stretching operation and resist a close fitting together of the same and a consequent full stretching of the leather. The mellowing process customarily employed in preparing leather for 35 stretching consists in soaking the leather in water. The resistance to stretching offered by the presence of the stuffing material in the leather is partly overcome by this water-soaking process but not to such an extent as 40 to permit a full stretching of the leather or the displacing of the stuffing material by the leather fibers. In other words, the water-soaking does not soften the stuffing material to such an extent that it becomes a yielding, 45 plastic or non-resistant substance so that it will yield easily to a drawing together of the fibers in the leather when subjected to a stretching strain.

The object of my invention is to so stretch 50 and treat leather preparatory therefor that the entire stretch may be taken out of the leather in a simple, thorough and efficient manner.

The invention is fully described in the 55 following specification, and while it is capable of being practised in numerous ways, a

preferred means for practising the same is illustrated in the accompanying drawings, in which—

Figure 1 is a perspective view of a cabinet 60 in which leather may be subjected to heat to mellow the same, a portion of the cabinet being broken away, and Fig. 2 is a perspective view of an apparatus for stretching the leather strips after being taken from the 65 mellowing cabinet.

In practising my process, leather strips of any desired size to be stretched are placed in the cabinet and preferably subjected to a steam or vapor heating treatment to soften 70 the stuffing material contained therein. In Fig. 1, 1 designates a cabinet which may be closed to render the same substantially steam-tight and which contains water 2 in its bottom portion and a false perforated or 75 lattice-work bottom 3 above the water 2 in which the leather strips 4 may be stood in edgewise position. A gas burner 5 or other suitable heating means is disposed below the cabinet to effect a heating of the water 2. 80 The heat within the cabinet is raised to a sufficient temperature to reduce the stuffing material contained in the leather to a plastic, yielding or non-resistant state, and inasmuch as different stuffing materials re- 85 quire different temperatures to soften the same, no specific temperature can be given for the heating of the leather. The heat usually employed, however, for mellowing the stuffing material of leather is around 90 110° Fahrenheit. Some materials, however, for instance, lard, will melt at a very much less degree of heat so that no fixed rule can be laid down for the temperature to be employed. The main thing to be borne in mind 95 in this connection is that only sufficient heat is required to render plastic the kind of stuffing material used.

It is preferable to employ a steam or wet heat, as better results are obtained than when 100 employing a dry heat for mellowing the stuffing materials contained in the leather.

When the leather has been sufficiently mellowed in the heat bath the strips are taken out as desired and subjected to a stretching 105 operation, as illustrated by the stretching apparatus shown in Fig. 2, any suitable type of which may be employed. This stretching is performed while the leather is in its heated or mellow state so that the fibers are 110 permitted to be drawn closely together during the stretching operation and to displace

the stuffing material, thus permitting the entire stretch to be taken out of the leather. When the stretching has been completed the leather is left on the stretcher until it cools sufficiently for the stuffing materials to congeal or assume a permanent set form, the time required for this in a warm room being approximately fifteen minutes. When the leather is stretched after the ordinary water mellowing process it is necessary to leave it on the stretching device until it dries, which requires several hours.

The advantages of my improved mellowing process over those heretofore used preparatory to stretching leather may be enumerated as follows:

First. The stuffing material offers a minimum of resistance to the stretching action.

Second. There is no loss of stuffing material as in the water-soaking process.

Third. The time required for stretching and a permanent setting of the stretched leather is materially shortened.

Fourth. The stretching can be more easily and thoroughly performed.

Fifth. Less space for handling and less labor required.

I wish it understood that my invention is not limited to the details described and to the use of apparatus of the class described

but is capable of numerous modifications without departing from the spirit of the claims.

Having thus described my invention, what I claim as new, and desire to secure by Letters Patent, is—

1. The process of stretching strips of heavy stuffed leather such as used for harness tugs, which consists in first applying heat to the leather to render the stuffing material therein plastic and yielding, then stretching the leather lengthwise of the strips while in a heated state thereby causing an exudation of stuffing material from the leather, and then allowing the strips to cool and set while under tension.

2. The process of stretching strips of heavy stuffed leather such as used for harness tugs, which consists in first applying wet heat to the leather to render the stuffing material therein plastic and yielding, then stretching the leather lengthwise of the strips while in a heated state thereby causing an exudation of stuffing material from the leather, and then allowing the strips to cool and set while under tension.

In testimony whereof I have hereunto signed my name to this specification.

IRVING H. ELLSWORTH.

Copies of this patent may be obtained for five cents each, by addressing the "Commissioner of Patents, Washington, D. C."